

Jan. 27, 1931.

R. H. ADAMS ET AL

1,790,494

METHOD OF MAKING LINSEED OIL

Filed July 3, 1925

2 Sheets-Sheet 1



Jan. 27, 1931.

R. H. ADAMS ET AL

**1,790,494**

## METHOD OF MAKING LINSEED OIL

Filed July 3, 1925

2 Sheets-Sheet 2



INVENTORS.  
Robert H. Adams  
Benjamin H. Durman  
Gifford & Scull  
ATTORNEYS.

## UNITED STATES PATENT OFFICE

ROBERT H. ADAMS, OF GREENWICH, CONNECTICUT, AND BENJAMIN H. THURMAN, OF TUCKAHOE, NEW YORK, ASSIGNEES TO GOLD DUST CORPORATION, OF NEW YORK, N. Y., A CORPORATION OF NEW JERSEY

## METHOD OF MAKING LINSEED OIL

Application filed July 3, 1925. Serial No. 41,275.

Our invention relates to method of making linseed oil.

Among the many uses to which linseed oil is put in the arts are two, namely, for varnishes and zinc grinding which require a very high-grade product. The ideal oil for these purposes must be of light color and is preferably brilliant without any bloom. Such an oil must also be free from what is known in the art as "break" when heated to a temperature substantially higher than 525° F. or when cooled to say 32° F. These breaks in the ordinary oil are evidenced by a precipitate which will not be re-dissolved upon cooling from the higher temperature or upon warming from the lower temperature. The presence of these precipitates in the oils as heretofore made, makes it necessary for the varnish or other paint maker to age and filter the oil before using it. The ideal oil should also be free of colored unsaponifiable residue, the unsaponifiable residue preferably being white or almost so. Such an oil should have a high viscosity and should have quick bodying properties with which a larger amount of thinner may be used than oils as heretofore made. Such an oil should also have a low phosphorus content, preferably less than one two-thousandth of one percent. The low phosphorus content assures the formation of phosphatides during the process of manufacturing products in which the oil is used. Such an oil should also be of such character that upon heat bleaching the color will be sufficiently light for use in the manufacture of varnish or in zinc or lead grinding. Preferably there should be no necessity for refining the oil by the use of caustics, acids, or other chemicals.

Linseed oil as heretofore made has had certain defects which it has been impossible to overcome prior to our invention. Two of the greatest defects have been the color and the breaks upon heating to 525° F. or higher, and upon cooling to 70° F. or lower. So far as we are advised no one prior to our invention has disclosed how these defects may be overcome without at the same time creating other defects somewhat less objectionable, but

materially decreasing the effectiveness of the oil.

Efforts have been made heretofore to overcome the objectionable color of the oil by treating the same with various chemicals, such as alkalis, acids, and others, and while this treatment has been successful to a certain extent as to color, these chemicals have so affected the structure or composition of the oil that the oil breaks when cooled, as above explained. The precipitate resulting from the breaks renders it necessary for the consumer of the oil to allow the same to remain in storage ordinarily for a period of six months. During this period the temperature of the oil changes according to the seasons and the precipitate settles in the barrels or other containers. When it is desired to use the oil it is then passed through a filter to remove this precipitate and clarify the oil. If it were attempted to use the oil before this aging period, these precipitates would be formed in the oil after the same had been made into varnish or other paints with the result that the paint or varnish would be objectionable and in fact unusable on high-class jobs. It therefore becomes necessary that the oil be stored to allow the precipitate to form and settle. Some varnish manufacturers have installed refrigerating apparatus to carry the oil through the necessary changes of temperature to facilitate the precipitation, in order to avoid this long period of aging. Obviously the aging is objectionable from several standpoints, among which may be mentioned the large amount of capital tied up in the material in storage, as well as the storage space and other equipment necessary therefor. The art has therefore been seeking for some time a solution of this difficulty which will relieve it of the dilemma of either storing the oil or of using the same with the chance that the product made therefrom will be defective because of the precipitated matter.

We have made certain discoveries and have devised a process of making a linseed oil free from all the defects above set forth and an oil which is superior to the best aged oil existing heretofore and an oil which may be used immediately upon production without the

necessity for any chemical treatment whatever, and at a lower cost than the best oils as heretofore made.

We have discovered that one of the chief causes of defects to the oil as heretofore made is the action of the constituents of the foreign matter which is invariably mixed with the flaxseed from which the oil is extracted. This foreign material is usually designated as dockage and consists of seeds of wild mustard, foxtail, vetch, white mustard, false flax, pigweed, clover and grass; also dust, grit, chaff, etc. Of course this dockage will contain other material and seeds of other plants depending upon the section of the country or world from which the seeds are gathered. Another substantial cause of the defects in the oil as heretofore made, was that of improperly controlled heat during the extraction of the oil from the seeds. We have discovered that if thoroughly clean flaxseeds are treated as heretofore wherein the temperature is not limited to below about 110° F., the resulting oil has most of the defects above mentioned. One of the chief defects is the break upon heating. On the other hand, it makes no difference what method is used to extract the oil from the seed, if the seeds have not been previously cleaned, the above-mentioned defects will appear.

Our new process consists in first cleaning the seeds of dockage so that there will remain in the seeds preferably not more than 1% to 1½%, preferably the former, of dockage. These seeds are then placed in an expeller and the oil expelled therefrom by cold pressing. That is to say, the expulsion of the oil is so regulated that the temperature of the oil running from the screen to the drip-pan is between 90 and 100 degrees F. Ordinarily this operation results in the expulsion of about 45 to 50% of the oil content of the seeds within the temperature range above given. The cake from which this oil has been expelled is then treated by an hydraulic press operation in any known way to remove the balance of the oil. The oil coming from the expellers may contain slight traces of moisture and fine particles of meal. In order to remove this material a quantity of the oil is run into and fills a tank of about five to six barrels capacity. To this about 100 pounds of diatomaceous earth is added and the mixture is thoroughly agitated with air. This mixture is then run into a filter press. This small quantity mixed with the diatomaceous earth causes the formation of a filter layer on the filter units and then a large quantity of the untreated oil may be run through the filters, which assures a very clear and brilliant oil. This oil after filtering shows about .60 acid number, color 50 yellow, 5.3 red. This oil as it comes from the filter has many uses and is particularly useful in the manufacture of var-

nish and is equal in color and other properties to the best varnish oil on the market which has been chemically treated and bleached. This oil is given in the table below as TA oil.

The oil from the filter may be treated in a very simple manner, that is to say, by heat, bleaching alone or by bleaching with earth, whereupon its color will be greatly reduced and an oil made which is particularly suitable for making light-colored varnishes or for zinc-grinding or other similar purposes. As an example of the heat bleaching, we have found that if 125 cc. of the above described TA oil are put into a 250 cc. beaker and heated to 600° F. in 10 minutes and held at this temperature for 15 minutes, the color is 17 yellow, 2 red, making a reduction in color of 33 yellow, 3.5 red. This oil is the ideal oil described at the beginning of this specification, having all of the qualities there mentioned without any defects, and in the table below is designated as P. M. P. oil.

We have noted that when oil made by ordinary methods is chilled to 60° F. or lower a cloudiness sometimes appears and does not disappear until the oil is at a temperature higher than that at which the cloudiness appeared. But with our oil a cloudiness does not appear until the temperature is 32° F. or lower. When a cloudiness appears, it will disappear before the temperature rises to 48° F., indicating that any suspended matter (such as glycerides crystallized out) caused by the chilling is soluble in the oil at the temperature of 48° F. or lower.

This bleached oil has a third use and that is that of making light fatty acids. These fatty acids are usually used for making driers or salts of drier metals. They are also used for increasing the acid content of any oil used in either zinc-grinding or lead-grinding. Such acids, as made from ordinary linseed oil, either raw or refined, have the great disadvantage of being of a dark color. This is objectionable if it is desired to use the acids to increase the acid content of a grinding oil, because of a tendency to discolor the product. By employing the bleached oil of our process fatty acid may be made of light color. When used to increase the acid content of an oil, these fatty acids may be merely added to the oil without treating the total quantity of oil as is usually done by the addition of sulphuric acid, heating and bleaching, which operation obviously consumes considerable time, and is rather expensive. Even if this expensive method is used, the resulting oil is many times darker in color than that made from the use of fatty acids which were made from our bleached oil.

From the foregoing it will be evident that we have devised a method by which a product is made which is much lighter in color than any similar product heretofore made; is en-

70

75

80

85

90

95

100

105

110

115

120

125

130

tirely free from suspended colloidal matter or precipitates which are not readily soluble in the material upon change of temperature: the material does not break when heated to a 5 high temperature or cooled to a low temperature; has a high viscosity and quick bodying properties; requires no refining by chemicals and therefore contains substantially all of its natural constituents; has a low phosphorus 10 content; will produce fatty acids of unusually light color and may be used as a varnish oil or as a grinding oil in the production of the highest grade paint products.

In the accompanying drawings, we have 15 indicated in Fig. 1 a flow sheet giving a diagrammatic representation of apparatus which we have used in the process above described. We wish it to be understood that this apparatus is by no means the only apparatus 20 which may be used in our process, but that it is merely representative.

We have shown in Fig. 2 an enlarged view of a seed cleaning machine somewhat in detail.

25 In Fig. 3 we have shown a view of the expeller on a larger scale than that shown in Fig. 1.

Our invention will be better understood by reading the following description of the 30 drawings forming a part thereof.

Referring to Fig. 1, the apparatus consists of a bin 1 for seed storage. The seeds are conducted from the bin 1 to the seed cleaners 2, 3 and 4. In treating flaxseed we have found 35 what is known in the trade as a No. 8 Monitor cleaner, made by the Huntley Manufacturing Company of Silver Creek, N. Y., very effective for our purpose. The cleaners 2 and 3 are of the type above indicated and each is 40 provided with a 16 x 2 1/2 inch wire screen and a 4/64 of an inch perforated metal screen for mustard seed fraction of the dockage. By running the seed over these cleaners the dockage is reduced to about 1.6 per cent. The 45 cleaner 4 is what is known in the trade as a No. 6 Monitor cleaner. This cleaner is provided with a mustard screen made up of a metal plate perforated to 4/64 of an inch. When the seeds are run over this cleaner they 50 are cleaned of dockage down to about 1 per cent or less.

Connected with each of the cleaners above described is a dust collector 5, 6 and 7, respectively. After the seed has passed over 55 these three cleaners it is conveyed into a hopper 8. The rough dockage is discharged at 9 and the mustard seed fraction of the dockage at 10.

The clean seeds are conveyed from the hopper 8 into the cracking or flaking machine 11. This is a two-high roll machine with the rolls so adjusted as to just flake or crack the hulls without grinding the hulls with the meats. This machine is driven at a speed of about 65 180 R. P. M. and is provided with means for

adjusting the rolls to regulate the cracking. From this machine the cracked or flaked seeds are delivered to the mixer 12 in which moisture is mixed with the seeds to the extent of about 3 per cent. An agitating means 13 is 70 shown for insuring a thorough mixing. The seeds mixed with this moisture are conducted by screw conveyor 14 to the expellers. The pressing equipment consists of a plate press 15, a box press 16 and a standard expeller 17. 75 By ordinary manipulation these pressers are operated so as to expel from the seeds about 45 to 50 per cent of the oil without raising the temperature of the oil as it leaves the expellers to a point higher than 90 to 110° F. 80 The oil is conveyed from the expellers to a scale tank 18 where the oil is weighed. Five or six barrels of oil are conducted into the pre-coating tank 19 in which the oil is mixed with about 100 pounds of a certain filter aid, such as diatomaceous earth. The oil and filter aid are thoroughly mixed by air agitation and the mixture is then run into the filter press 20, whereupon the filter aid forms a coating on the filter elements, thus assuring a complete filtering of the oil which is later run through. 85

From the filter press the oil is run into testing tanks 21 and 22 and is there tested for quality before being delivered to the storage tank 23. 90

The test of the oil in the tanks 21 and 22 consists in removing a sample from the tank and testing the acid number and the color of the oil. In our operation the acid number runs between .58 and .6 and the color from about 50 yellow and 7 red to about 35 yellow, 5 1/2 red. The color measurements herein given were determined by the Lovibond colorimeter with 5 1/4 inch column and used in the 100 customary manner. 105

The oil that is delivered to the tank 23 has many uses, as explained in the first part of this specification, but for many purposes we find it advisable to further treat the oil by passing it into the bleaching tank 24, in which is placed an agitator 25. A steam pipe 26 is placed in the bleach tank and by means of steam the temperature of the oil in the tank 24 may be controlled to any desired point. 110 We prefer to maintain the temperature in the tank 24 at about 180° F. 115

We prefer to add to the oil in the tank 24 about 3 1/2 per cent fuller's earth and 1/6 of 1 per cent of a suitable carbon bleaching material. After the addition of the earth and the bleaching material the oil is pumped through the filter press 27. At the beginning of the operation it is customary to return the oil from the filter press to the bleaching tank 120 until a sufficient bed or cake of filter material is built up on the press units. After the filter press is properly prepared the oil is run continuously from the filter press into a storage tank 28. The oil coming from the filter press 125 130

27 has a color ranging from about 10 yellow and 1 red, to about 20 yellow and 2 red, and an acid number of about .5.

We have shown in Fig. 2 a somewhat more detailed view of the seed cleaning machine. This machine per se forms no part of our invention and we therefore do not deem it necessary to fully illustrate and describe the same. The machine consists of a framework 5 supporting a series of screens 30, 31, 32, 33. These screens are reciprocated by eccentrics 34 and 35 on a shaft 36. The material to be cleaned is introduced through the receptacle 37 at one end of the machine or receptacle 38 at the other, or both at the same time. The foreign matter is removed by means of the fan 29 and the cleaned flax seeds are delivered at 40. The mustard seeds are delivered at 41, and the screenings at 42. This 10 machine is well known in the art and its operation is thoroughly familiar to those acquainted with the cleaning of flaxseed.

In Fig. 3 we have shown a standard expeller which is operated by motor 43 and acts to expel the oil from the cracked flaxseed by compressing the seed between the plates 44. The oil is delivered at 45 and the cake or solid matter may be discharged at 46 from the expeller in a well-known manner. This machine is also well known to those skilled in the art and its construction and operation need no further description.

The following table gives the ranges of values of the various physical characteristics of crude oil made in the ordinary way and of the oil as it comes from the tank 23 (TA oil) and of the oil in the tank 28 (P. M. P. oil).

|    |                       |                    |  |  |  |  |
|----|-----------------------|--------------------|--|--|--|--|
| 40 | Oil                   | Raw                |  |  |  |  |
|    | Color                 | 300 yellow, 22 red |  |  |  |  |
|    | Acid No               | 0.6 to 4.0         |  |  |  |  |
|    | Viscosity             | 1½ seconds         |  |  |  |  |
|    | Iodine No             | 180 to 198         |  |  |  |  |
| 45 | Gravity               | .932 to .934       |  |  |  |  |
|    | F. F. A.              | .3% to 2.0%        |  |  |  |  |
|    | Unsaponifiable matter | Not over 1.50%     |  |  |  |  |

| 50 | Oil | Color              | Acid No. | Viscosity  | Iodine No. | Gravity      |
|----|-----|--------------------|----------|------------|------------|--------------|
|    | TA  | 35y—5.3R<br>50y—7R | .6 to 1  | 1½ seconds | 180 to 198 | .932 to .934 |
|    | PMP | 10y—1R<br>20y—2R   | .6 to 1  | 1½ seconds | 180 to 198 | .932 to .934 |

| 60 | Oil | F. F. A. | Refractive index | Bodying rate | Unsaponifiable matter | Phosphorus content |
|----|-----|----------|------------------|--------------|-----------------------|--------------------|
|    | TA  | .3 to .5 | 1.4793           | 1 to 5 hrs.  | .1.07                 | Less than .001     |
|    | PMP | .3 to .5 | 1.4792           | 1 to 4 hrs.  | .76                   | Less than .002     |

65 While we have given details such as the

color and acid number of the product and other details as to the method of treatment, we desire to have it understood that we are not limited to these exact figures as many changes may be made and satisfactory results produced, but we have found that the method above described in detail is the preferred commercial method and that the product identified above is entirely suitable for all commercial purposes.

Throughout the specification and claims the term "viscosity" and the values thereof given or indicated, are determined by the "bubble method," as follows: The instrument consists of a glass tube 6" long by  $\frac{3}{8}$ " in diameter. The tube is sealed at one end and is made in the form of a homeopathic vial so that it can be almost filled with oil or other material and sealed at the open end with a cork stopper. The tube is filled with oil or other material to such an extent that when the stopper is inserted the air bubble when allowed to flow along the side of the tube is  $\frac{1}{3}$  the diameter of the tube, i. e. it is  $\frac{1}{8}$ " in diameter. The viscosity is determined by first bringing the air bubble completely to one end of the tube and then inclining the tube suddenly at an angle of 60° and measuring with a stop watch or other suitable means, the time required for the transit of the bubble to the other end of the tube. This determination is made at a temperature of approximately 70° F. The above instrument and method of determining viscosity thereby are well known in the art and have been used for many years and form no part of this invention.

It may be found necessary to change the method of treatment to a slight degree depending upon the character of the seed used and the section of the country or world from which the seeds came, but in view of the foregoing disclosure, we believe that those skilled in the art can easily and readily adapt the process to the treatment of any seeds by very slight experimentation.

We claim:

1. The method of extracting linseed oil which consists in cleaning the whole un-cracked flaxseed to a maximum of about 1.5% dockage and pressing the oil from the cracked flaxseed while limiting the upper temperature of the oil below 110° F.

2. The method of extracting linseed oil which consists in cleaning the whole un-cracked flaxseed to a maximum of about 1.5% dockage and pressing a portion only of the oil from the cracked flaxseed while limiting the upper temperature of the oil below substantially 110° F.

3. The method of extracting linseed oil which consists in cleaning the whole un-cracked flaxseed to a maximum of about 1.5%

dockage and pressing not more than substantially 45% to 50% of the oil content of the seed from the cracked flaxseed while limiting the upper temperature of the oil below substantially 110° F.

R. H. ADAMS.  
BENJAMIN H. THURMAN.

10

15

20

25

30

35

40

45

50

55

60

65